

# United States Patent Office

2,717,832

Patented Sept. 13, 1955

1

2,717,832

## DIAZOTYPE MATERIALS FOR BLACK LINE IMAGES CONTAINING DIRESORCYL SULFIDE OR SULFOXIDE AS A SUBSTITUTE FOR RESORCINOL

John Sulich, Jr., Endicott, N. Y., assignor to General Aniline & Film Corporation, New York, N. Y., a corporation of Delaware

No Drawing. Application September 8, 1954,  
Serial No. 454,837

5 Claims. (Cl. 95-6)

The present invention relates to diazotype materials capable of being processed to black images, and more particularly to the utilization in the formation of such materials of diresorcylic sulfide or diresorcylic sulfoxide as a substitute for resorcinol as a coupling component.

It is common practice in the diazotype field to produce images which are of different colors, such as blue, red, sepia and the like. The desirability for materials which may be processed to produce images simulating black in color is self-evident. However, the production of such materials is not a simple matter for the simple reason that there is not available one coupling component capable of reacting with a light sensitive diazonium compound under alkaline conditions to yield a black image.

There are available on the market diazotype materials which are capable of being processed to black images. However, all such materials contain at least three coupling components, i. e., one which yields a yellow-green image, another which yields a blue image, and a third, normally considered a shading component, which yields a yellow-brown image.

In the past it has been customary to employ resorcinol as the shading component, acetoacetanilide to give the yellow-green image and 2,3-dihydroxy naphthalene-6-sulfonic acid to yield the blue image. The mixture of the dyes obtained with these coupling components, when in admixture on paper, results in a reasonably black color in the maximum densities and a desirable greenish-gray in the lower tones.

It is recognized that the storage of diazotype materials, particularly under warm humid conditions, results in a differential migration of the chemicals into the fibrous base on which they are coated. This is particularly true with respect to resorcinol which, because of its relatively low molecular weight and high water solubility, is very susceptible to migration into the fibrous base and away from the light sensitive diazonium compound. It has been my experience that black line diazotype materials formulated with resorcinol as the only shading component, when stored, yield, upon printing and developing, images which are too bluish in color due to the absence of the brown shade caused by the migration of resorcinol. It has also been my experience that it is difficult, if not impossible, to distinguish such prints from the ordinary blue line diazotype prints. Needless to say, customer complaints and rejects of the sensitizing paper are customary with such diazotype materials.

It has now been discovered that a storage stable black line diazotype material, free from the objections previously noted, can be obtained by replacing the resorcinol in whole or in part by either diresorcylic sulfide or diresorcylic sulfoxide. It was ascertained that neither of these compounds showed any appreciable tendency to diffuse into the fibrous base. As a matter of fact, whereas previously humidity-aged prints (to simulate natural shelf storage of several months) showed a color shift to the

2

blue due to the diffusion of resorcinol, similarly aged prints containing diresorcylic sulfide or diresorcylic sulfoxide with or without resorcinol remained a neutral black.

Black line diazotype materials containing as the coupling components a mixture of acetoacetanilide and 2,3-dihydroxy naphthalene-6-sulfonic acid with diresorcylic sulfide or diresorcylic sulfoxide, with or without resorcinol, as the brown shade constitute the purposes and objects of the present invention.

10 Diresorcylic sulfide and diresorcylic sulfoxide have the following respective formulae:

Diresorcylic Sulfide



Diresorcylic Sulfoxide



15

20

25

30

35

40

45

50

55

60

65

70

Both of these components are known compounds and methods of their preparation are available in the literature. It is recommended, however, that the sulfide be prepared by reacting sulfur dichloride in ether with resorcinol in ether at a temperature not higher than 12° C., neutralizing the reaction solution with sodium carbonate, stripping the ether from the organic layer and crystallizing the sulfide from water.

In the event that the sulfoxide is to be employed, it may be prepared from the water-wet sulfide by suspending the same in water at 65° C., and oxidizing the sulfide with an excess of hydrogen peroxide at 65-75° C.

It is a typical feature of black line diazotype materials that the mixture of the coupling components used must each have a low coupling speed. If this were otherwise the material would have poor shelf life due to premature coupling of any component having high coupling power. It is to be noted, in this connection, that satisfactory black line papers cannot be produced by using such high speed couplers as 2,3-dihydroxy naphthalene, phloroglucinol and the like. For practical purposes I have found it to be essential to use with the diresorcylic sulfide or sulfoxide, as the case may be, acetoacetanilide to give the yellow-green image and 2,3-dihydroxy naphthalene-6-sulfonic acid to give the blue image. These components have the low coupling speed required and in addition furnish with the brown shade on the fibrous base. Resorcinol may also be present to complement the shading action of the diresorcylic compound and to preclude any possibility of a shift in the image color to red.

More latitude is allowed in the selection of the light sensitive diazonium compound than in the selection of the coupling components. Thus, it is possible to use any light sensitive diazonium compound which is derived from a p-phenylenediamine. Examples of such light sensitive diazonium compounds are those from N-diethyl-p-phenylenediamine; N-dimethyl-p-phenylenediamine; N-dipropyl-p-phenylenediamine; N-ethyl-N-β-hydroxyethyl-p-phenylenediamine; N-methyl-β-hydroxyethyl-p-phenylenediamine and the like. According to customary practice it is preferred to use these diazonium compounds in the form of their stabilized double salts with a metal halide, such as zinc chloride, aluminum chloride, tin tetrachloride and the like.

## 3

The coating solution, in addition to the coupling components and the light sensitive diazonium compound, may also contain the various adjuncts usual in the manufacture of light sensitive diazotype materials. These include metal salts for intensification of the dyestuff image, such as ammonium sulfate, nickel sulfate, zinc chloride and the like; stabilizing agents such as thiourea, thiosinamine, naphthalene trisulfonic acid and the like; acids acting to retard precoupling such as acetic acid, boric acid, tartaric acid and the like; hygroscopic agents such as glycol, glycerin and the like; and wetting agents such as saponin, lauryl sulfonate, ketyl benzene sulfonate, the oleic acid amide of N-methyl taurine and the like.

The base to which the coating solution is applied may be any fibrous base which has been previously suggested for employment in the diazotype field. Examples of such bases are high grade all-sulfite bond paper, rayon or cotton cloth, starch filled cloth and the like.

It is believed to be evident from the formulae of the diresorcylic derivatives contemplated herein that neither 20 has a structure which is high in molecular weight. Furthermore, each possesses a plurality of hydroxyl groups which would tend to render the two compounds soluble in water. The non-diffusibility of these derivatives, therefore, cannot be predicated either on high molecular 25 weight or water insolubility of the products.

It is my opinion that the non-diffusibility of the diresorcylic compounds is attributable to the formation of a complex with the diazonium compound employed. Thus, it could be envisaged that one molecule of the diresorcylic 30 sulfide would form the following complex with two molecules of the zinc chloride double salt of the diazo from N-diethyl-p-phenylenediamine:



Similarly, it is presumed that one molecule of diresorcylic sulfide would form the following complex with one molecule of the aforementioned diazonium compound:



It is to be emphasize that no positive proof has been developed to support this theory. However, it is a fact that related compounds, such as 2,2',4,4'-tetrahydroxybi-

phenyl; 2,4,4'-trihydroxybiphenyl and various condensation products of resorcinol with formaldehyde, on the one hand, and phosgene, on the other hand, were much closer to resorcinol in their tendency to diffuse than the diresorcylic compounds contemplated herein.

This leads me to believe that my theory is correct although it is to be understood that the possibility of the formation of a complex is only a theory and one which is offered merely for the sake of explaining the otherwise inexplicable results which I have attained.

The following examples will serve to further illustrate the invention, but it is to be understood that the examples are illustrative only.

## Example I

An all sulfite bond paper was coated with the following solution and dried:

|                                                                      |                            |
|----------------------------------------------------------------------|----------------------------|
| Water                                                                | 60 cc.                     |
| Glycol                                                               | 5 cc.                      |
| Isopropanol                                                          | 1 cc.                      |
| Citric acid                                                          | 8 grams.                   |
| Zinc chloride                                                        | 5 grams.                   |
| Thiourea                                                             | 5 grams.                   |
| Diresorcylic sulfide                                                 | 1.3 grams.                 |
| Acetoacetanilide                                                     | 0.26 gram of 26% strength. |
| 2,3 - dihydroxynaphthalene - 6 - sulfonic acid                       | 1.8 grams.                 |
| Zinc chloride double salt of diazo from N-diethyl-p-phenylenediamine | 3.2 grams.                 |
| Saponin                                                              | 0.1 gram.                  |
| Water to                                                             | 100 cc.                    |

The above paper, even when stored for a period of several months in a humid atmosphere, gave, upon printing and development with ammonia gas, prints which were of a neutral black shade.

## Example II

The procedure is the same as in Example I, excepting 40 that the diresorcylic sulfide is replaced by an equimolecular quantity of diresorcylic sulfide. The results, obtained upon storage, printing and developing the resulting paper, were substantially the same as in Example I.

## Example III

The procedure is the same as in Example I, excepting that the light sensitive diazonium compound is the zinc chloride double salt of the diazonium compound from N-ethyl-N-β-hydroxyethyl-p-phenylenediamine which is 50 employed in an amount equivalent to the sensitizer in Example I.

The product obtained is comparable in properties to the product of the preceding examples.

## Example IV

The procedure is the same as in Example I, excepting that there is used one gram of diresorcylic sulfide and 0.8 gram of resorcinol.

The paper compounded in this fashion yielded prints 60 of a neutral black even after storage for a considerable period in a humid atmosphere.

## Example V

The procedure is the same as in Example I, excepting 65 that diresorcylic sulfide is replaced by 0.6 gram of diresorcylic sulfide and there is added 1.2 grams of resorcinol.

Prints made with the resulting paper simulated those of Example IV.

70 It may be noted at this point that the proportions of active ingredients, to wit, coupling components and light sensitive diazonium compound appearing in the examples, are not critical. Thus, it is possible to vary the quantity of these components 10% either plus or minus the figures given in the examples, particularly when

the absorbency of the paper coated is taken into consideration.

The present application is in part a continuation of my application Serial No. 383,406, filed September 30, 1953, now abandoned, entitled "Diazotype Materials for Black Line Images Containing Diresorcy1 Sulfide or Sulfoxide as a Substitute for Resorcinol."

Various modifications of the invention will be apparent to operators in this field, and I, therefore, do not intend to be limited in the patent granted except as necessitated by the appended claims.

I claim:

1. A storage stable light sensitive diazotype material capable of producing black azo dye images upon printing and development comprising a fibrous base coated with a light sensitive diazonium compound of the p-

10

15

phenylenediamine class and a mixture of coupling components comprising acetoacetanilide, 2,3-dihydroxy naphthalene-6-sulfonic acid and a diresorcy1 derivative selected from the class of diresorcy1 sulfide and diresorcy1 sulfoxide.

2. The product as defined in claim 1, wherein the diresorcy1 derivative is diresorcy1 sulfide.

3. The product as defined in claim 1, wherein the diresorcy1 derivative is diresorcy1 sulfoxide.

4. The product as defined in claim 1, wherein the light sensitive diazonium compound is derived from N-diethyl-p-phenylenediamine.

5. The product as defined in claim 1, in which the mixture of coupling components includes resorcinol.

No references cited.